

- [54] **PROCESS FOR THE DYEING OF TOW IN HYDRATED CONDITION**

[75] Inventors: **Gottfried Eigenmann, Therwil; Leo E. Kaiser, Aesch; Otto Nöthiger, Oberwil, all of Switzerland**

[73] Assignee: **Ciba-Geigy AG, Basel, Switzerland**

[22] Filed: **Oct. 31, 1972**

[21] Appl. No.: **302,504**

#### **Related U.S. Application Data**

- [63] Continuation of Ser. No. 150,754, Dec. 22, 1970, abandoned.

**[30] Foreign Application Priority Data**

- Dec. 23, 1969 Switzerland..... 19173/69

- [52] U.S. Cl. .... 8/177, 8/151  
[51] I. 1. Cl. .... D26-2/72

- [51] Int. Cl. .... D06p 3/70  
[58] Field of Search 8/151.2 151.1 177 177 AB

- [58] **Field of Search** ... 8/151.2, 151.1, 177, 177 AB,  
8/1 151; 68/181 R

[ 56 ] References Cited

UNITED STATES PATENTS

- 2,558,735 7/1951 Creswell ..... 264/28

- |           |         |                 |          |
|-----------|---------|-----------------|----------|
| 2,949,337 | 8/1960  | Oldershaw ..... | 8/15/1.2 |
| 3,241,343 | 3/1966  | Yazawa.....     | 68/181 R |
| 3,315,501 | 4/1967  | Muller.....     | 68/181 R |
| 3,353,381 | 11/1967 | Taylor.....     | 68/181 R |

*Primary Examiner*—Leon D. Rosdol

*Assistant Examiner—T. J. Herbert, Jr.*

*Attorney, Agent, or Firm—E. F. Wenderoth et al.*

[57]

## ABSTRACT

A process for the continual dyeing of fibres produced by a wet spinning process, in particular for the continual dyeing of polyacrylonitrile tow in a hydrated condition is disclosed in that the fibre or the fibre strand after fibre formation without previous drying is passed through a dyestuff solution or suspension which is flowing in counter current. Said process is very economical and provides without the use of any electronic controls the continual dyeing of said fibres with almost 100 percent exhaustion.

## 1 Claim, 2 Drawing Figures



PATENTED JAN 22 1974

3,787,182



FIG. 1



FIG. 2

INVENTORS  
GOTTFRIED EIGENMANN  
LEO E. KAISER  
OTTO NÖTHIGER

BY *Wendworth, Lind & Ponack*  
ATTORNEYS

## PROCESS FOR THE DYEING OF TOW IN HYDRATED CONDITION

This is a continuation of application Ser. No. 100,754, filed Dec. 22, 1970, now abandoned.

Polyacrylonitrile fibres are produced by the so-called dry spinning process in which the fibre is produced from polymers dissolved in organic solvents by evaporating the solvent, or they are obtained by the so-called wet spinning process in which the fibre is precipitated in aqueous solution with the addition of electrolytes. In the so-called wet spinning processes, directly following the actual fibre-forming process (spinning process), the fibre is first subjected to several washings and then to a stretching process in order to orientate the macromolecules before it is dried. In this "swollen" condition, the fibre is to a very high degree capable of absorbing the dyestuff, e.g. in an aqueous bath. In this state the dyeing can thus be performed under substantially milder conditions than are necessary for dyeing the same fibre after the spinning process when the fibre has been dried. Thus dyeing of tow in a hydrated condition saves energy and time; in addition a drying process can be eliminated.

Processes for the dyeing of fibres in a gel-like condition which hitherto have been known consist essentially of bringing the fibres in contact with the dyestuff solution either on a padding mangle or in a simple dyebath and then washing hot. Since in a continuous process, dyestuff is continually being removed from the dyebath, in the known processes specific measures must be taken to guarantee a constant concentration of dyestuff in the dyebath in order to obtain a specific shade. Such operations as, e.g. measuring the concentration of the dyestuff and regulating the additional amounts of concentrated dyestuff required, e.g. by means of an electronic regulating arrangement are unavoidable. When a dyestuff mixture is employed, as is usually the case, it is necessary to dose the additional amounts of the several dyestuffs individually according to their dyeing behaviour and thus the individual dyestuff solutions must be controlled separately. Such regulating arrangements are very complicated and expensive, and often the dosed amounts tend to vary.

It has now surprisingly been found that fibres produced by wet spinning processes, in particular polyacrylonitrile tow, can be continually dyed in a hydrated condition in a simple manner by passing the fibre, or fibre strand, after its formation and without drying it, through a dyestuff solution which is flowing in counter current. This counter current principle is, for example, known in so-called cascade washers in the production of fibres.

The application of the counter current principle to the dyeing of tow in a hydrated condition is very economical. Furthermore, without the use of any electronic controls, it permits the continuous dyeing in a simple manner of the said fibres in specific shades and with almost 100 percent exhaustion.

The process can, for example, be performed in an apparatus which is characterized by a series of communicating containers; a means for conveying the fibre strands through these containers; a means for feeding the dyestuff solution, which means opens into the last container relative to the direction of conveyance; the containers being equipped with baffle plates which di-

rect the flow of the dyestuff solution in the direction opposite to the path of conveyance.

Such an arrangement is illustrated, for example, more in detail in the drawing:

FIG. 1 shows (in a diagrammatic representation in section) an example of an embodiment of the apparatus according to the invention for the performance of the counter current dyeing, and

FIG. 2 shows a section along the line II — II of FIG. 1.

The dyeing aggregate shown consists essentially of a series of containers  $S_1, S_2 \dots S_n$ , a conveying device G,H for fibre strands F leading through these containers, a mixer L for the preparation of the dyestuff solution, and a proportioning pump K. The outlet of the mixer is connected via the proportioning pump with the last container  $S_n$  relative to the direction of conveyance. The containers  $S_n, S_{n-1} \dots S_1$  communicate with each other via overflow channels D. Baffle plates C which force the dyestuff solution to flow in the direction opposite to the path of conveyance are mounted in the containers. The first container is provided with an outlet E which is preferably a type of overflow. M designates a double jacketed heating means controlled by a thermostat for the series of containers.

This dyeing aggregate functions as follows.

The supply of mixed dyestuff solution in mixing tank L is passed after optional dilution via the proportioning pump K to point A of the last container of the dyeing aggregate. The solution is forced by the baffle C in counter current direction to flow downward past point B and then at point D of the last container into the next to last container. The liquor then passes through all of the containers in the same manner and finally leaves the first container at point E. The fibre material, which has received the usual treatment after the spinning process, comes from point F over the guiding rollers G and H and is dipped into the first container. The time spent in this container is determined on the one hand by the speed of the conveyance of the fibre and on the other hand by the dimensions of the individual containers. It should be in the order of from about 0.1 to 30 seconds. The fibre is thus brought into contact with the last concentrated dyestuff solution, absorbs a certain amount of dyestuff, then moves on to the next container where the dyestuff concentration is higher. In this manner at the end of the nth container, the fibre comes in contact with fresh dyestuff solution so that after an equilibrium has been attained, the depth of shade of the material leaving at point I is constant. The guiding roller G and H should be constructed in such a manner that the tow is spread out as widely as possible when passing through the individual containers in order to obtain an optimal penetration of the dyestuff solution in the tow.

The depth of shade is controlled on the one hand by varying the concentration of the dyestuff solution in mixing tank L and on the other hand by varying the amount of solution dosed by proportioning pump K. With a constant concentration in tank L and a constant dosing, there is an equilibrium of the concentration in the individual containers, which decrease from container (n) to container (n-1 ... 1). The optimal adjustment is reached when the concentration of the dyestuff solution leaving at point E is zero or at least almost zero, since in this manner an almost complete utilization of the dyestuff is attained. The time required until equilibrium is reached depends on the size of the indi-

vidual containers, the smaller the volume of the containers, the less time is needed. Since the velocity of the dyeing process as well as the equilibrium of the concentrations attained on the fibre depend on the temperature of the dyebath, it is advantageous to surround the entire dyeing aggregate with a jacket M which is controlled by a thermostat. For the performance of the dyeing of hydrated polyacrylonitrile tow, it should permit a constant temperature to be kept in the range between 20 and 70°C.

The advantage of the new dyeing process described are that the dyestuff employed can be practically completely utilized and that there is no fluctuation of the depth of shade of the material leaving at I, such as is the case with systems depending on the measurement of a value and a regulation derived from that measurement (additional dosing). In addition the problems of uneven end results are avoided, since each section of the fibre material comes in contact with fresh dyestuff solution at the end of the dyeing process.

The dyebaths usual in practice may be used in the process according to the invention. It is convenient to prepare them by dissolving or dispersing the dyestuff in water and adjusting the pH of the dyebath obtained with an acid and/or a buffer salt to the desired value.

Disperse dyestuffs as well as anionic and in particular cationic dyestuffs may be used according to the invention. Dyestuffs of any class may be used.

Disperse dyestuffs which may be used according to the invention are preferably azo dyestuffs, as well as antraquinone, nitro, methine, styryl or azostyryl dyestuffs.

Suitable as anionic dyestuffs in the process according to the invention are any class of the so-called acid wool dyestuffs as well as of substantive dyestuffs in which the coloring constituent is in the anion such as the alkali or ammonium salts of dyestuff sulphonic or carboxylic acids, i.e. metal-free or metallized sulphonated mono-azo or disazo dyestuffs, in which are also included the formazane dyestuffs, their chromium, cobalt, nickel and copper complexes, as well as sulphonated anthraquinone, nitro and phthalocyanine dyestuffs.

Cationic dyestuffs which may be used according to the invention are advantageously the technically easily obtainable salts and metal halides, for example the zinc chloride double salts, of known basic dyestuffs. These are, for example, dyestuffs containing onium groups such as thiazines, oxazines, diphenyl methanes, tri-phenyl methanes, rhodamines, azo and anthraquinone dyestuffs, preferably monoazo, methine, azomethine

and anthraquinone dyestuffs, the onium groups being preferably ammonium groups.

The following examples illustrate the invention. Temperatures are given therein in degrees centigrade.

#### Examples

Dyeing is performed in a dyeing aggregate consisting of five elements S<sub>1</sub> to S<sub>5</sub> connected in series, constructed in such a way that the tow has a dip time of 0.7 second per element when it is passing at a rate of 0.5 meter per second. This corresponds to a dip length of 0.35 m/element. Such an aggregate is illustrated in FIG. 1, the individual elements S<sub>1</sub> to S<sub>5</sub>, however, are arranged in cascade form.

The dyeing aggregate is continually charged at G with polyacrylonitrile tow which has been produced from a solution of polyacrylonitrile in sodium thiocyanate by the wet spinning process, and has been stretched, as is usual in industry, at 95°, then washed but not dried. The water content of the tow is reduced by squeezing out the excess to about 170 percent of the dry weight. The amount of tow entering the dyeing aggregate at G can be seen in Table II.

An aqueous solution is a dyestuff, the composition of which is given in Table II, is mixed in feed tank L, and then mixed in a constant proportion with the proportioning pump K in a T-shaped mixing element together with a constant proportion of water, and introduced at A to element S<sub>5</sub>, care being taken that the dyestuff solution is spread over the complete width of the apparatus.

The tow which enters the elements S<sub>1</sub> to S<sub>5</sub> at G in a colorless state is successively dyed in the individual elements and is completely dyed as it leaves the aggregate at I.

The dyestuff solution which has remained on the tow is removed by two squeezing rollers and discarded. The dyed tow is then rinsed for a short time in hot water and then dried. The concentration of the dyestuff solution slowly decreases from element S<sub>5</sub> to S<sub>1</sub>, so that the dyestuff solution leaving the aggregate at E is colorless or almost colorless.

If, when the aggregate is put into operation, the elements are first all filled with water, an equilibrium of the dyestuff concentration is reached in the individual elements after several minutes. After equilibrium has been reached, when the dosing rate and the dosing concentration remain constant, the shade of the dyed tow remains constant even over a long period of time.

The following Table I gives the structures of the dyestuffs used:

TABLE I  
I Dyestuff of the formula



II Dyestuff of the formula



## III Dyestuff of the formula



## IV Dyestuff of the formula



## V Dyestuff of the formula



## VI Dyestuff of the formula



## VII Dyestuff of the formula



## VIII Dyestuff of the formula



## IX Dyestuff of the formula



The following Table II gives the components used in Examples 1 to 9, the amounts thereof and the dyeing conditions used. At the end of each Example, the shade of the polyacrylonitrile fibre dyed according to the invention is given.

TABLE II

| Dyestuff                        | Examples      |               |               | Dosage, water                                           | 850<br>ml/min | 800<br>ml/min | 800<br>ml/min |
|---------------------------------|---------------|---------------|---------------|---------------------------------------------------------|---------------|---------------|---------------|
|                                 | 1             | 2             | 3             |                                                         |               |               |               |
| Concentration of stock solution | 43 g/l        | 43 g/l        | 43 g/l        | Water temperature                                       | 30°C          | 800<br>ml/min | 800<br>ml/min |
| Acetic acid, conc.              | 2 g/l         | 2 g/l         | 2 g/l         | Temperature in Elements S <sub>1</sub> - S <sub>5</sub> | 38-32°C       | ca. 25°C      | ca. 25°C      |
| Sodium acetate, conc.           | 2 g/l         | 2 g/l         | 2 g/l         | Amount of polyacrylo-                                   | 430<br>g/min  | 38-26°C       | 37-25°C       |
| pH                              | 4.6           | 4.6           | 4.6           | nitrile tow                                             |               |               |               |
| Temperature                     | 30°C          | 30°C          | 30°C          | Relative dyestuff concentration*                        |               |               |               |
| Dosage, stock solution          | 110<br>ml/min | 110<br>ml/min | 110<br>ml/min | in equilibrium                                          |               |               |               |
|                                 |               |               |               | Element S <sub>5</sub>                                  | 92 %          |               |               |
|                                 |               |               |               | Element S <sub>4</sub>                                  | 56 %          |               |               |
|                                 |               |               |               | Element S <sub>3</sub>                                  | 35 %          |               |               |
|                                 |               |               |               | Element S <sub>2</sub>                                  | 18 %          |               |               |
|                                 |               |               |               | Element S <sub>1</sub>                                  | 8 %           | ca.           | ca.           |
|                                 |               |               |               | Squeezed solution removed                               | 2.4 %         | 2 %           | 2 %           |
|                                 |               |               |               |                                                         | 0.2 %         | ca.           | 2 %           |

|                                            |        |        |        |
|--------------------------------------------|--------|--------|--------|
| Exhaustion                                 | 91 %   | 98 %   | 98 %   |
| Depth of shade attained**                  | 4.4 %  | 0.24 % | 0.13 % |
| Shade of the dyed poly-acrylonitrile fibre | yellow | grey   | blue   |

Keys

\* conc. at introduction = 100%

\*\* Dyestuff calculated on the weight of the dry fibre

The following two optical brighteners were used in Examples 10 and 11 given in the following Table III. The components in the amounts used are given in this Table III as well as the conditions of the treatment and the optical brightening results obtained. The procedure is otherwise the same as described in Example 1.

## X Optical brightener of the formula



## XI Optical brightener of the formula



|                                                         | Examples              |                    |                        |
|---------------------------------------------------------|-----------------------|--------------------|------------------------|
|                                                         | 7                     | 8                  | 9                      |
| V :<br>35 g/l                                           | VII :<br>88 g/l       | VIII :<br>12.6 g/l |                        |
| <b>Dyestuff</b>                                         | <b>VI :<br/>7 g/l</b> |                    | <b>IX :<br/>62 g/l</b> |
| Concentration of stock solution                         | -                     | -                  | -                      |
| Acetic acid, conc.                                      | -                     | -                  | -                      |
| Sodium acetate, conc.                                   | -                     | -                  | -                      |
| pH                                                      | 6.8                   | 6.4                | 6.4                    |
| Temperature                                             | 48°C                  | 25°C               | 55°C                   |
| Dosage, stock solution                                  | 165                   | ml/min             | 110                    |
| Dosage, water                                           | 700                   | ml/min             | ml/min                 |
| Water temperature                                       | 55°C                  | 1250               | ml/min                 |
| Temperature in Elements S <sub>1</sub> - S <sub>5</sub> | 42-53°C               | 30°C               | ml/min                 |
| Amount of polyacrylo-                                   | 430                   | 35- 28°C           | 55°C                   |
|                                                         | g/min                 | 430                | g/min                  |
| Relative dyestuff concentration**<br>in equilibrium     | ca. 6 %               | 4 %                | ca. 8 %                |
| Element S <sub>5</sub>                                  | -                     | 66 %               | -                      |
| Element S <sub>4</sub>                                  | -                     | 41 %               | -                      |
| Element S <sub>3</sub>                                  | -                     | 25 %               | -                      |
| Element S <sub>2</sub>                                  | -                     | 16 %               | -                      |
| Element S <sub>1</sub>                                  | -                     | 11 %               | -                      |
| Squeezed solution removed                               | ca. 86 %              | 88 %               | ca. 84 %               |
| Exhaustion                                              |                       |                    |                        |
| Depth of shade attained**                               | 1.4 %                 | 1.96 %             | 0.87 %                 |
| Shade of the dyed poly-                                 | green                 | red                | orange                 |
| acrylonitrile fibre                                     |                       |                    |                        |
| Key:                                                    |                       |                    |                        |
| * conc. at introduction = 100%                          |                       |                    |                        |
| ** Dyestuff calculated on the weight of the dry fibre   |                       |                    |                        |

The present process is also suitable for the optical brightening of fibres which have been produced by a wet spinning process. Dispersable anionic and, in particular, cationic optical brighteners are suitable for use in the process according to the invention. Various classes of these brighteners may be used. Especially brilliant optical brightening effects are obtained with anionic compounds derived from the stilbene class and with cationic compounds derived from the coumarin class.

TABLE III

|    |                                                                | Examples    |             |
|----|----------------------------------------------------------------|-------------|-------------|
| 25 | Optical brightener                                             | 10          | 11          |
|    | Concentration of stock solution                                | X           | X           |
|    | Acetic acid, conc.                                             | 4 g/l       | 5 g/l       |
|    | Sodium acetate, conc.                                          | 0.5 g/l     | —           |
|    | pH                                                             | 0.5 g/l     | —           |
| 30 | Temperature                                                    | 4.6         | 6.2         |
|    | Dosage, stock solution                                         | 30°C        | 40°C        |
|    | Dosage, water                                                  | 110 ml/min  | 140 ml/min  |
|    | Water temperature                                              | 1700 ml/min | 1400 ml/min |
|    | Temperature in Elements S <sub>1</sub> -S <sub>3</sub>         | 25°C        | 50°C        |
|    | Amount of polyacrylonitrile tow                                | 36-25°C     | 48-42°C     |
|    | Relative concentrations * of optical brightener in equilibrium | 430 g/min   | 430 g/min   |
| 35 | Element S <sub>3</sub>                                         | 56 %        | 58 %        |
|    | Element S <sub>4</sub>                                         | 36 %        | 42 %        |
|    | Element S <sub>3</sub>                                         | 20 %        | 25 %        |
|    | Element S <sub>2</sub>                                         | 6 %         | 7.2 %       |
|    | Element S <sub>1</sub>                                         | 2 %         | 2.6 %       |
| 40 | Squeezed solution removed                                      | <0.2 %      | <0.2 %      |
|    | Exhaustion                                                     | 98 %        | 96 %        |
|    | Optical brightening effect **                                  | 0.1 %       | 0.15 %      |
|    | Treated polyacrylonitrile fibre                                | white       | white       |
|    |                                                                | brightened  | brightened  |

**Key:**

\* conc. at introduction = 100%

\*\* Optical brightener calculated on the weight of the dry fibre

### **What we claim is:**

1. A process for the continuous dyeing of a polyacrylonitrile fiber or fiber strand in a hydrated condition, produced by a wet spinning process, after fiber formation but without being previously dried, which comprises passing said fiber or fiber strand through a dye-stuff solution or suspension following in countercurrent, wherein a dye solution or suspension of constant concentration is introduced at constant rate at the place where the fiber leaves the dyestuff solution or suspension and the relative velocity of the fiber to the dyestuff solution or suspension is so adjusted that at that point where the fiber enters the dyestuff solution or suspension, the dyebath has a concentration of zero, or substantially zero, and the dyeing is performed at a constant temperature in the range between 20 and 70°C.